

O. L. MILLS,  
PROCESS OF UNITING ALLOY STEEL TO CARBON STEEL,  
APPLICATION FILED OCT. 10, 1919.

1,376,963.

Patented May 3, 1921



FIG. 1.



FIG. 3.

WITNESS:

P. F. P. Hutchel.

INVENTOR

Oscar L. Mills

BY

Frank J. Buser  
ATTORNEY.

# UNITED STATES PATENT OFFICE.

OSCAR L. MILLS, OF EASTON, PENNSYLVANIA.

## PROCESS OF UNITING ALLOY STEEL TO CARBON STEEL.

1,376,963.

Specification of Letters Patent. Patented May 3, 1921.

Application filed October 10, 1919. Serial No. 329,750.

*To all whom it may concern:*

Be it known that I, OSCAR L. MILLS, a citizen of the United States, residing at Easton, county of Northampton, and State 5 of Pennsylvania, have invented a new and useful Improvement in Processes of Unit- 10 ing Alloy Steel to Carbon Steel, of which the following is a full, clear, and exact de- 15 scription, reference being had to the accom- 20 panying drawings, which form a part of this specification.

It is well known that various steel alloys have certain wear-resisting or shock-resist- 15 ing qualities, such as hardness, toughness 20 and the like, which render them superior to high grades of carbon steel in the manufac- 25 ture of articles intended for a wide variety of uses. On the other hand, such alloy steels are relatively very expensive, and in the 30 manufacture of various articles, especially those of which only a small part is exposed to excessive wear or wherein it is necessary for only the surface of the article to have the superior quality sought, it is uneconomical to manufacture the entire article from 35 an expensive alloy. In these cases, and also in any case wherein it is desirable that the body of the article should be composed of carbon steel, efforts have been made electri- 40 cally, with unsatisfactory results, to apply a permanent superficial coating of alloy steel to ordinary carbon steel or to integrally secure to a body of carbon steel a 45 wearing part of alloy steel.

35 A known method of procedure is by electric welding with an alloy steel rod used as one electrode. This method has certain pronounced advantages, but it is open to serious objection. As is well known, alloy 40 steel usually has a substantially lower melting point than low carbon steel, and hence, during the passage of the current, the steel alloy melts and flows over the surface of the carbon steel before the latter can be 45 raised to the melting temperature. The result is that the adhesion between the carbon steel and the steel alloy is imperfect and in actual use the connection between the two is apt to be ruptured, thus destroy- 50 ing the utility of the compound article.

The object of my invention is to devise a process wherein, by the aid of the electric welding, a body of alloy steel, or other alloyed metal, in the shape of a superficial 55 coating for an article of iron, steel, or other

metal body having a higher melting point than the alloyed metal, or as a distinctive part or element of the complete article, may be as securely united to said body as in the case of the welding together of two pieces 60 of metal of the same melting point, whereby the alloyed metal will be integrally and permanently united to said body. More specifically, the process involves the manufac- 65 ture of the alloyed metal coincidentally with the welding thereof to said body, as herein- 70 after more specifically detailed.

In the drawings, which are illustrative of a preferred way of uniting an alloy steel to a body of low carbon steel: 70

Figure 1 is a side view showing diagrammatically a way of carrying out my process.

Fig. 2 is a view showing the process of making the compound rod or pencil used in my process. 75

Fig. 3 is an enlarged cross-sectional view of such rod.

I first proceed to manufacture, by casting, rolling, or otherwise, a rod *a*. I prefer to manufacture this rod of steel low in car- 80 bon and therefore with a high melting point.

The said rod is then inclosed in a body *b* of material composed of the metal or metals which it is desired to incorporate 85 with the steel to form the alloy steel, thus forming a rod or electrode of which the rod *a* constitutes the core.

I prefer to manufacture the compound rod by reducing the metal or metals *b* to a 90 finely divided condition, impregnating them with linseed oil or another suitable binder, spreading the impregnated mass on a wrapper *c* of linen or other fabric, inclosing the core *a* with the alloys and their wrapper, 95 and baking, or in some cases air-drying, the same until the body *b* reaches the condition of a hard mass.

The compound rod *a b* is then brought close to the surface of the body of steel *d* 100 to which the alloy steel is to be united, the steel *d* and the rod *a b* being connected to opposite poles of an electric circuit. A tem- 105 perature sufficient to melt the approximating end of the electrode also suffices to melt the approximating surface of the steel. The steel core *a* and the alloying metals *b* melt and combine to form an alloy steel and as they melt they are projected upon a steel sur- 110 face that has also become molten, thus caus-

ing an indissoluble union between the steel body and the alloy steel.

The invention is of course not limited to the manufacture of compound articles wherein the alloyed metal is of any particular composition, and therefore no attempt will be made to enumerate all the metals capable of use as alloys: As examples may be mentioned manganese, nickel, cobalt, 10 chromium, vanadium and tungsten, or two or more of these associated together. Such alloying metals will ordinarily be themselves alloys, as, for example, ferro-manganese, ferro-vanadium, etc.

15 Having now fully described my invention, what I claim and desire to protect by Letters Patent is:

1. The process of uniting a metal coating with the surface of a metal body, comprising 20 the steps of coating a tape with a paste containing the alloying material in a finely divided state, wrapping the coated tape about a metal core with the coated side in contact with the core to form an electrode, then drying the electrode, and then passing an electric current through the electrode and the 25 metal to be coated, to fuse the end of the electrode and the surface of the metal body

to be coated to unite the fused alloy with the fused surface of the metal body.

2. The process of making electrodes for uniting with a metal body, comprising the steps of coating a tape with a paste containing finely divided alloying metals, wrapping said tape about a metal core to form the 35 electrode, and then drying the electrode.

3. The process of making electrodes for uniting with a metal body, comprising the steps of making a paste of linseed oil and finely divided alloying metals, evenly spreading the paste on an insulating tape, then wrapping the tape about a metal core to form an electrode, and then drying the electrode.

4. An electrode comprising a steel core, an 45 even coating of alloying material mixed with linseed oil, and an outer covering of tape.

5. An electrode comprising a low carbon steel core with a high melting point, an even coating of alloying material mixed with linseed oil, and an outer covering of tape.

In testimony of which invention, I have hereunto set my hand, at Philadelphia, Pa., on this 4th day of October, 1919.

OSCAR L. MILLS.